

June 12, 1923.

W. L. WOODWARD

1,458,605

METHOD OF MAKING SEAMLESS TUBES RICH IN ZINC

Filed Feb. 21, 1921

Fig. 1



Fig. 2



Fig. 3



Fig. 4



Fig. 5

Inventor  
W. L. Woodward

By  
Kline Brock & West  
Attns.

Patented June 12, 1923.

1,458,605

# UNITED STATES PATENT OFFICE.

WILLIAM L. WOODWARD, OF LAKewood, OHIO.

## METHOD OF MAKING SEAMLESS TUBES RICH IN ZINC.

Application filed February 21, 1921. Serial No. 446,649.

*To all whom it may concern:*

Be it known that I, WILLIAM L. Woodward, a citizen of the United States, residing at Lakewood, in the county of Cuyahoga and State of Ohio, have invented a certain new and useful Improvement in Methods of Making Seamless Tubes Rich in Zinc, of which the following is a full, clear, and exact description, reference being had to the accompanying drawings.

This invention relates to a novel method for making seamless tubes of zinc or of an alloy rich in zinc.

The object of the invention is to provide a cheap and simple method of producing seamless tubes of the composition mentioned which shall possess ductility and malleability so that the said tubes can be drawn, bent, swaged or otherwise manipulated as desired.

With this object in view the invention consists in the steps hereinafter explained in detail and set forth in the appended claims.

In the drawings I have diagrammatically outlined the steps of my process and in which Fig. 1 is a longitudinal and a transverse cross section of a tubular body in the first stage of fabrication; Fig. 2 is a similar view indicating the second stage or step; Fig. 3 is a longitudinal and a cross sectional view of the finished tube and Figs. 4 and 5 are longitudinal sectional views of tubes drawn from the finished tube indicated in Fig. 3.

In carrying out my invention I provide a seamless tubular body A preferably of zinc, or of an alloy or compound rich in zinc.

This seamless tubular body A may be made by casting in any suitable manner or it can be produced by extrusion or said seamless tubular body can be produced by casting a solid ingot and then boring the same.

This seamless tubular body of zinc or a compound rich in zinc possesses a well defined crystalline structure or formation and in carrying out my improved method this crystalline structure or formation is broken up or the molecular structure of the seamless tubular body is transformed so as to render the same ductile and malleable. This change or transformation I propose to make by mechanically treating the crystalline tubular body and it will be understood that there are a variety of such mechanical treatments such as hammering, rolling and swaging and in the drawing I have shown the crystalline tubular body A placed upon

a suitable mandrel B and subjected to the action of a hammer C, this mechanical treatment in the form of hammering, serving to completely change the molecular formation so that the crystalline formation is completely broken up and the tubular body as a whole rendered ductile and malleable and in Fig. 3 I have indicated diagrammatically the tubular body D in which such transformation or change has taken place. The crystalline tubular body having been transformed into a ductile and malleable tubular body can be readily drawn after the well known methods and in Figs. 4 and 5 I have shown the tube illustrated in Fig. 3 in successive steps of drawing. A seamless tube made in accordance with the above method can be drawn or bent and can be treated, utilized or fabricated in any manner in which any seamless tube possessing ductility and malleability can be utilized and treated.

The method above described has the advantage of simplicity and cheapness and at the same time provides a seamless tube of exceptional merit.

It will thus be seen that I provide a simple and highly efficient method by means of which a seamless tube of material rich in zinc and possessing ductility and malleability can be provided.

Having thus described my invention, what I claim is:

1. The herein described method of making seamless tubes of material rich in zinc which consists in first producing a crystalline tubular body of a material rich in zinc and then mechanically treating said tubular body to break up the crystalline structure thereof and render said tubular body ductile and malleable.

2. The method of making seamless tubes of the kind described, which consists in providing a tubular body of a material rich in zinc and of crystalline structure, and then mechanically changing the molecular structure of said tubular body and rendering the same malleable and ductile.

3. The method of making seamless tubes of the kind described, which consists in making a tube rich in zinc and a crystalline structure, then mechanically treating said tube to transform the molecular structure thereof so as to render said tube ductile and malleable.

4. The method of making seamless tubes

of the kind described, which consists in first providing a seamless zinc tube of crystalline structure and then mechanically treating said tube to break up the crystalline formation and produce a seamless zinc tube, the molecular structure of which possesses the qualities of ductility and malleability.

5. The herein described method of trans-

forming a crystalline tubular body rich in zinc into one possessing the properties of 10 ductility and malleability, which consists in mechanically treating said tubular body to effect a rearrangement of the molecules.

In testimony whereof, I hereunto affix my signature.

WILLIAM L. WOODWARD.